

## 1

3,011,881

 NOVEL BORON COMPOUNDS AND MOTOR FUEL  
CONTAINING THE SAME

Donald D. Emrick, Shaker Heights, Chien-wei Liao, Beachwood, and Edwin O. Hook, Chagrin Falls, Ohio, assignors to The Standard Oil Company, Cleveland, Ohio, a corporation of Ohio  
No Drawing. Filed May 3, 1960, Ser. No. 26,439  
6 Claims. (Cl. 44-63)

This invention relates to novel boron compounds and to motor fuels containing the same. More particularly, this invention relates to a class of boron compounds which serve as excellent multi-functional additives in a gasoline for a spark-ignited internal combustion engine.

The boron compounds of the present invention have the following general formula:



where X is hydrogen or



and wherein R represents a radical selected from a group consisting of alkyl, alkenyl, or alicyclic radicals containing from 7 to 21 carbon atoms, and R' is selected from a group consisting of hydrogen or an alkyl radical containing up to 5 carbon atoms.

Gasolines containing one or more of the compounds of the present invention are effective in markedly reducing many of the adverse effects resulting from combustion chamber deposits which accumulate during the prolonged operation of an initially clean engine on a hydrocarbon fuel, and particularly a hydrocarbon fuel which contains tetraethyl lead as an octane improver. One of the most serious adverse effects of lead deposits is uncontrolled ignition and a general lack of smoothness in engine operation caused principally by these deposits becoming heated to incandescence within the combustion chamber during engine operation and igniting the fuel either before or after the portion in the cycle at which the charge would normally be ignited by the spark of the sparkplug. The boron compounds of the present invention are helpful in overcoming in great part this adverse effect of lead deposits.

It is well known that organoboron compounds are effective in minimizing engine operating problems due to deposits, but many of the boron compounds previously proposed for such use are not suitable in commercial practice due to the characteristic instability of organoboron compounds toward hydrolysis while in gasoline. Because of this instability, contact with small amounts of water and moist, atmospheric conditions during prolonged storage causes many of the prior art compounds to hydrolyze to solid insoluble products which precipitate out of the gasoline phase, so that the boron content never reaches the engine where it might be effective. In contradistinction to this general characteristic of boron compounds, the compounds of the present invention are quite stable toward hydrolysis while in gasoline and are well suited for conventional large scale manufacturing and marketing operations.

Additionally, gasolines containing boron compounds

## 2

of the present invention are highly effective in minimizing carburetor icing, usually making it unnecessary to incorporate a special additive in the gasoline to guard against this problem. Carburetor icing represents a troublesome problem attendant to automotive engines operated in cool, moist, atmospheric conditions. This icing problem is most likely to occur during engine warmup when the engine is below normal operating temperature. The vaporization of the gasoline in the carburetor during this warmup period produces temperature reduction in the throttle plate and carburetor walls, causing the moisture present in the incoming air on cool, humid days to condense and freeze. Such ice formation restricts the narrow openings in the carburetor, manifesting itself in a rough idling condition and frequent engine stalls.

The gasoline base stocks to which the present boron compounds are added may be any of those conventionally used in preparing a motor gasoline for a spark-ignited internal combustion engine, such as catalytic distillate, motor polymer, alkylate, catalytic reformate, isomerate, naphthas, etc. The gasoline will preferably contain a tetra alkyl lead compound as an anti-knock agent and a scavenging agent. The amount of anti-knock agent will usually be at a level of approximately 3 ml./gal. but may range from  $\frac{1}{2}$  ml./gal. up to 6 ml./gal. The base gasoline may also include other common additives such as anti-oxidants, stabilizers, solvent oils, dyes, and the like.

30 The amount of the boron compound added to the fuel may vary and the amount is preferably expressed in terms of boron. Generally an amount of the compound to provide 0.002% by weight of boron (based on the total fuel) is the smallest amount that will give any significant effect. Use of amounts in excess of 0.1% by weight of boron usually cannot be justified economically. These compounds may be added directly to the fuel or, if more convenient, they may be dissolved in a suitable solvent to produce a liquid concentrate and the concentrate blended in with the fuel.

35 The compounds of the invention are prepared by reacting boric acid with a mono-acylated trialkanol amine compound in an equimolar relationship. The mono-acylated trialkanol amine compounds employed in this reaction may be characterized by the following general formula:



40 wherein R and R' are defined as hereinbefore. The latter compounds are preferably prepared by reacting a trialkanol amine compound with a fatty acid or naphthenic acid compound containing 8 to 22 carbon atoms in a 1:1 molar ratio under conditions to remove the water of reaction that is formed. Compounds prepared by reacting triethanol amine or triisopropanol amine with oleic acid are particularly desirable for the gasoline compositions of the present invention. Commercial grades of the preferred fatty acids which are derived from naturally occurring fats and oils are suitable for the reaction, and hence the R radical in the above formula may correspond to the fatty acid radicals present in such fats and oils. The R radical may also be suitably derived from naphthenic acids containing from 8 to 22 carbon atoms.

45 50 55 60 65 70 The mono-acylated trialkanol amine compound readily undergoes boration under conditions in which the water of reaction is removed from the reaction mixture as it

is formed. The reaction proceeds in accordance with the equation:

(I)



or the equation:

(II)



depending upon the amount of water that is removed during the reaction.

substance which was readily soluble in gasoline. The product has the formula:



The water of reaction may be removed by simple boiling but it is preferable to remove the water by means of azeotropic fractional distillation using preferably benzene, toluene, or xylene as the solvent. Boric oxide may be used in place of the boric acid as the boron source in the above reactions with the proper adjustment of the molar relationship with the mono-acylated trialkanol amine compound.

The preparation of these compounds will be better understood in connection with the following examples.

#### Example 1

56.5 grams (0.2 mole) of oleic acid was mixed with 38.3 grams (0.2 mole) of tri-isopropanol amine in the presence of 80 ml. of xylene. The reaction mixture was heated with stirring at the azeotropic distillation temperature until 3.2 ml. of water of reaction was removed (3.6 ml. represents theoretical or 0.2 mole).

12.4 grams (0.2 mole) of boric acid was then added to the mono-acylated amine and the reaction mixture was heated again to azeotrope out 2.0 moles of water for each mole of mono-acylated amine and boric acid reacting. The reaction mixture was filtered and the excess solvent was then removed. The resulting product was a transparent viscous material which was completely soluble in gasoline. The product has the following formula:



#### Example 2

141 grams (0.5 mole) of oleic acid was mixed with 95.8 grams (0.5 mole) of tri-isopropanol amine together with 300 ml. of benzene in a three-necked flask. This reaction mixture was heated with stirring at the azeotropic distillation temperature to remove 8.8 ml. of water (9.0 ml. represents theoretical or 0.5 mole).

31 grams (0.5 mole) of boric acid was then added to the flask containing the mono-acylated amine and the reaction mixture was heated again to the azeotropic distillation temperature and maintained under these conditions until 2½ moles of water of reaction was removed for each mole of mono-acylated amine and boric acid reacting. The excess solvent was then removed from the reaction mixture and the product was a clear plastic

substance which was readily soluble in gasoline. The product has the formula:

The following tests were conducted to show the benefits available by the use of these compounds in gasoline with respect to suppressing surface ignition and protecting against carburetor icing.

To illustrate the improvements toward surface ignition suppression, tests in an ASTM-CFR single cylinder engine having a compression ratio adjusted at 12:1 were employed. Preparatory to the test cycle the engine was run open throttle at 900 r.p.m. for 30 minutes to stabilize the engine conditions for the test period. Following this, the engine was operated at open throttle continuously for three hours, during which time the total surface ignition count was observed electronically. All experimental conditions were the same for each test except the gasoline.

The base fuel in each test was the same and had the following composition and specifications.

##### Composition:

|    |                            |              |
|----|----------------------------|--------------|
| 60 | 62% Ultraformate           |              |
|    | 20.9% cat. distillate      |              |
|    | 2.9% lt. naphtha           |              |
|    | 6.5% lt. alkylate          |              |
|    | 4.2% isopentane            |              |
|    | 3.5% butane                |              |
| 65 | Tetraethyl lead            | ml./gal. 2.4 |
|    | API gravity                | 57.8         |
|    | Engler distillation, ° F.: |              |
|    | I.B.P.                     | 91           |
| 70 | 10%                        | 122          |
|    | 30%                        | 170          |
|    | 50%                        | 229          |
|    | 70%                        | 281          |
|    | 90%                        | 370          |
|    | E.P.                       | 426          |
| 75 | Reid vapor pressure        | 11.24        |



where X is selected from the group consisting of hydrogen and



and wherein R represents a radical selected from the group consisting of alkyl, alkenyl, and alicyclic radicals containing from 7 to 21 carbon atoms, and R' is selected from the group consisting of hydrogen and alkyl radicals containing up to 5 carbon atoms.

5. A novel boron compound having the following general formula: 15



where X is selected from the group consisting of hydrogen and



20

6. A novel boron compound having the following general formula:



10 where X is selected from the group consisting of hydrogen and



References Cited in the file of this patent

UNITED STATES PATENTS

|           |                |               |
|-----------|----------------|---------------|
| 2,741,548 | Darling et al. | Apr. 10, 1956 |
| 2,939,877 | Washburn       | June 7, 1960  |
| 2,942,021 | Groszos et al. | June 21, 1960 |
| 2,948,597 | Belden         | Aug. 9, 1960  |